

Dec. 3, 1963

E. J. LARSEN

3,113,020

METHODS OF IMPROVING EXTRUSION PROPERTIES  
OF LEAD-ANTIMONY ALLOYS  
Filed July 19, 1961



FIG. 1



FIG. 2



INVENTOR.  
E. J. LARSEN  
BY *E. J. Larsen*  
ATTORNEY

## 1

3,113,020

## METHODS OF IMPROVING EXTRUSION PROPERTIES OF LEAD-ANTIMONY ALLOYS

Elmer J. Larsen, Parkville, Md., assignor to Western Electric Company, Incorporated, New York, N.Y., a corporation of New York

Filed July 19, 1961, Ser. No. 125,160

2 Claims. (Cl. 75—135)

This invention relates to methods of improving extrusion properties of lead-antimony alloys and more particularly to methods of improving extrusion properties of lead-antimony alloys for continuous extrusion in screw-type metal extruders.

In the manufacture of telephone cables, it has long been the practice to extrude lead-antimony alloys, preferably those containing about one percent of antimony by weight of alloy, as cable sheathing over a core of the cable. Such lead-antimony alloys were usually prepared by adding relatively pure antimony or a master alloy, containing about 22 percent of antimony by weight of the alloy to relatively pure lead. The mixture was heated to a temperature in the range of from about 700° F. to about 800° F. to melt the mixture to dissolve the antimony in the lead. The molten mixture was usually agitated to disperse the antimony or the master alloy relatively uniformly throughout the principal.

The melt was then cast into ingots and transferred to a location where it was desirable to extrude the lead-antimony alloy as a sheath over a cable core. When it was necessary to extrude the sheath, the ingots were heated to normal pre-extruding temperatures of from about 700° F. to about 800° F. to melt the ingots. The molten alloy was then extruded as a sheath upon a cable core by means of a conventional screw-type metal extrusion apparatus of the type disclosed in U.S. Patent 2,076,200, issued April 6, 1937, to R. E. Horley.

The area adjacent to the die of the extrusion apparatus was maintained at normal working or extrusion temperatures from about 390° F. to about 480° F., preferably at 450° F. However, it was observed that extrusion of such lead-antimony alloys prepared and extruded by the above methods presented various problems, such as stepwise separation of the cooling molten alloy into relatively antimony-poor solid portions and relatively antimony-rich liquid portions, resulting in surging of the molten alloy being extruded, stoppages of the extrusion apparatus caused by segregation of the alloy, and nonuniform composition of the extrudate.

An object of this invention is to provide new and improved methods of improving extrusion properties of lead-antimony alloys.

Another object of the invention is to provide new and improved methods of improving extrusion properties of lead-antimony alloys for continuous extrusion in screw-type metal extruders.

These objects are realized in accordance with the various aspects of the present invention by melting the lead-antimony alloy and then heating it to such a relatively high temperature that dross, formed at lower temperatures on top of the molten alloy and including primarily oxides of lead and antimony, is melted and the surface of the molten alloy takes on specular appearance.

A complete understanding of the invention may be obtained from the following detailed description of methods forming specific embodiments thereof, when read in conjunction with the appended drawings, in which:

FIG. 1 is a phase diagram for a lead-antimony system;

FIG. 2 is an enlarged view for a relatively low-antimony concentration portion of the diagram of FIG. 1, and

FIG. 3 is a diagram of a curve representing minimum

## 2

dross-melting temperature and composition relationship in a lead-antimony system.

Referring now in detail to the drawings, FIGS. 1 and 2 show a conventional phase diagram, or an equilibrium diagram as it is sometimes called, for a two component system, in this case, a lead-antimony system. The diagram shows the temperatures at which any specific lead-antimony alloy changes phase from solid to liquid and vice versa. Abscissa shows percentage of antimony by weight of composition in the system. The percentage of lead may be found at any point along the abscissa by simply subtracting the percentage of antimony from 100 percent. Ordinate gives the temperature for the various changes.

The phase diagram is composed of several lines which are Liquidus, Solidus and Solvus lines. Lead-antimony alloys of certain composition are liquid and completely fluid at the temperatures above the Liquidus lines. Lead-antimony alloys, the temperature of which is below the Liquidus lines, but above the Solidus lines, are in a pasty or semiliquid form, wherein one part of the alloy has frozen out of the melt resulting in a mushy or spongy substance. Lead-antimony alloys, the temperature of which is below the Solidus lines, are completely frozen and are composed of solids. A lead-antimony alloy which has a eutectic composition, i.e. about 11.2 percent of antimony by weight of alloy, changes sharply upon cooling, from liquid to solid at about 485.6° F. Similar, but opposite changes take effect upon heating of these alloys.

A lead-antimony alloy to be extruded, such as one containing from about 0.05 percent to about 10.2 percent, but preferably from about 0.1 percent to about 1.2 percent, of antimony by weight of alloy, is normally heated before extrusion to normal pre-extrusion temperatures from about 700° F. to about 800° F. The molten alloy is then fed into a working chamber of a conventional screw-type metal extrusion apparatus of the type disclosed in the above-identified patent to R. E. Horley. The alloy is then advanced by a screw impeller toward a die and extruded through the die to form the sheath about the cable core. Various parts of the apparatus may be heated or cooled to maintain the metal in various parts of the apparatus in desired molten, plastic or solid state. The die is maintained at normal extrusion temperatures of from about 390° F. to about 480° F., preferably of about 450° F.

As a result of this difference between the pre-extrusion and the extrusion temperatures of the alloy, a temperature gradient in the range of from about 220° F. to about 410° F. exists along the working chamber. When a lead-antimony alloy containing, for example, one percent of antimony is cooled from about 800° F. down to about 450° F. and the alloy is at rest, the cooling will follow a vertical line  $x-x$  (FIG. 2). When the line  $x-x$  intersects the Liquidus line at a point 11, which corresponds to temperatures of about 610° F., the melt begins to freeze. The material first to freeze is a material rich in lead and poor in antimony, i.e., the material indicated by a point 12 and having about 0.3 percent of antimony. The remaining liquid becomes enriched in antimony and has a lower freezing point, so that a point representing the concentration and temperature of the liquid remaining during the cooling follows down the Liquidus line. For example, at the temperature of about 600° F., about two-thirds of the original melt will be frozen as a material containing about 0.7 percent of antimony, while about one-third of the original melt will remain liquid and contain about 2 percent of antimony. The ratio of solid to liquid at any time during the freezing is determined by an inverted ratio length of levers formed by intersection of the line  $x-x$  with a horizontal line connecting Liquidus and Solidus lines for a particular temperature.

70

When the melt is cooled down to temperatures corresponding to a point 13, which is the point of intersection of the line  $x-x$  with the Solidus line and corresponds to temperatures of about  $580^{\circ}$  F., the liquid phase is no longer possible for this composition and all of the original melt will become solid. The last drop of alloy to freeze at this temperature will have composition corresponding to a point 14 on the Liquidus line which corresponds to about 3.3 percent of antimony. Any further cooling of the now solid alloy down to about  $450^{\circ}$  F. results in cooling of the solidified alloy to the desired extrusion temperature. The point 13 gives also the average composition of the melt which has solidified, which is one percent of antimony by weight of alloy.

The above freezing has been described as an empirical freezing which takes place when an alloy being cooled is at rest. A grain or a crystal starts its growth with a normally dendritic structure, the framework of which is composed of the purer material surrounded by the liquid which is richer in the alloying material, in this case antimony, so that a mushy or a spongy mass is formed filled with liquid which continues to freeze until the whole mass is frozen solid.

When the same material is agitated during cooling, for example, when the alloy is cooled within the extruding apparatus while being advanced by the screw impeller, the spongy material is kneaded whereby the liquid is separated from the solid part. During the extrusion, the frozen alloy portion is picked up by the screw impeller of the extrusion apparatus 11 and the liquid alloy portion rich in antimony is left behind, resulting in the separation of the original alloy into alloys of various instantaneous compositions similar to a zone refining separation process. The instantaneous remaining antimony-rich liquid alloy portion of the original lead-antimony alloy then is cooled in steps similar to those described hereinabove with reference to FIG. 2 for the alloy having one percent of antimony, but at lower temperatures depending on the composition of the remaining liquid. The separation continues until finally a liquid which has a eutectic composition, i.e., about 11.2 percent of antimony by weight, is left behind, which freezes last. Because of the tendency of the screw impeller of the extrusion apparatus to pick up the hard frozen material and leave behind the antimony-rich liquid alloy, the above separation has been found to result in certain difficulties, such as uneven cooling and surging of the material, irregular rates of extrusion and even complete stoppages of the extrusion of the material, stalling of the equipment during the extrusion, and variations in the composition of the extruded sheath.

The surging of the material has been found to occur because of the tendency of the screw impeller to churn the liquid antimony-rich portion of the alloy, remaining after the frozen antimony-poor portion thereof has been picked up by the screw impeller and has been forwarded toward the die, and then to pick up suddenly the remaining antimony-rich alloy. Such suddenly picked-up portion is usually the stepwise antimony-enriched, partially frozen antimony-rich portion of the alloy, which in some cases may even have been separated down to the eutectic composition. This lag in being picked up by the screw impeller is explained by a longer interval of time required to cool antimony-rich portions of the lead-antimony alloy. The stoppages of the material and, in many cases, stalling and stoppages of the equipment has been found to occur, primarily, due to the inability of the lead press to forward the suddenly picked-up frozen portion of the original lead-antimony alloy, particularly, when the separation of the alloy resulted in a relatively large amount of an alloy portion having eutectic or near eutectic composition, which freezes suddenly at about  $485.6^{\circ}$  F. to lock the screw impeller so as to prevent rotation thereof.

In accordance with the present inventions, the above-described difficulties may be obviated by a process of heat-treating at relatively high temperatures a lead-antimony

alloy, containing from about 0.05 percent to about 10.2 percent, preferably from about 0.1 percent to about 1.2 percent of antimony by weight of alloy prior to extrusion. According to this process, an alloy having a desired composition is heated until molten, and the molten alloy is heated to relatively high temperatures in the range from about  $1000^{\circ}$  F. to about  $1400^{\circ}$  F. The heating is continued until dross, which is formed on top of the molten alloy as a thin overlaying crust of lead and antimony oxides, disappears and the surface of the molten alloy takes on specular appearance.

The molten alloy may then be used for extrusion immediately after the dross-melting process by modifying, if necessary, the usual steps of the sheath-extrusion procedure so as to utilize the molten alloy the temperature of which is well above the normal pre-extrusion temperatures. Alternatively, the molten alloy may be cast into ingots and cooled. When needed for extrusion, the ingots are remelted to the usual pre-extrusion temperatures of the process (from about  $700^{\circ}$  F. to about  $800^{\circ}$  F.), in accordance with the usual continuous sheath-extrusion procedures. In both cases, the extrusion of such heat-treated lead-antimony alloy over the cable core proceeds continuously with resultant relatively uniform composition of the extruded sheath.

Without limiting the invention to any theory and merely for the purpose of facilitating the comprehension of the above-identified method, the following mechanism is proposed to explain the change in extrusion properties of the lead-antimony alloys in question. The dross, which consists substantially of lead oxides and antimony oxides, forms, upon melting, various eutectic compositions with the lead-antimony alloys, which could be represented by equilibrium diagrams (not shown) completely different from that for an alloy consisting only of lead and antimony. The molten dross is taken up into the liquid lead-antimony solution and is dispersed relatively uniformly throughout the solution. Upon cooling, the various dross-containing eutectic compositions freeze before the mass of the lead-antimony alloy begins to freeze and form a plurality of nuclei for the framework to form the sponge-like mass of antimony-poor portion of the alloy filled with the relatively antimony-rich liquid portion of the alloy. The so-formed sponge-like mass entraps this liquid to such an extent, that upon kneading by the screw impeller the liquid alloy portion is not separated from the relatively solid portion of the alloy but continues to freeze until the whole mass is frozen. It is also believed that this heat-treatment inhibits, to some extent, a normally dendritic growth of the metal crystals of the alloy so that a relatively smooth physical appearance of the frozen alloy is obtained. As a result of this heat-treatment, the above-mentioned problems were substantially eliminated, allowing utilization of presently available continuous-type extrusion apparatus for truly continuous extrusion.

The relationship between the dross-melting temperatures and compositions of relatively pure lead-antimony alloys are presented by a curve 16 of the dross-melting temperature and alloy composite graph shown in FIG. 3. Abscissa of the graph shown in FIG. 3 shows percentage of antimony by weight of composition in the system. Ordinate of the same graph gives the minimum dross-melting temperature for various compositions. For example, an alloy having about one percent of antimony, corresponding to a point 17 on the curve 16, should be heated to at least  $1095^{\circ}$  F. to melt the dross.

Examination of FIG. 3 shows that alloys having relatively low percentages of antimony, within the above-indicated range of compositions, require to be heated to higher minimum temperatures to melt the dross, and alloys having relatively high percentages of antimony within the same range may be heated to lower minimum temperatures within the above-indicated heating range to melt the dross, the minimum dross-melting temperature increasing substantially inversely proportional to a decreasing antimony content of the alloy.

The minimum dross-melting temperatures of the lead-antimony alloys may be below or above the melting temperature of a pure antimony (1166.7° F.), depending on the lead-antimony alloy composition. Examination of the curve 16 of FIG. 3 shows that lead-antimony alloys containing more than about 0.33 percent of antimony by weight of the composition may be heated below the melting temperature of pure antimony, i.e. below 1166.7° F. However, lead-antimony alloys containing less than about 0.33 percent of antimony by weight of the composition should be heated above 1166.7° F., the minimum dross-melting temperature increasing with decrease in the antimony content of the alloys.

In some cases it may be desirable to prepare an alloy of the type containing from about 0.05 percent to about 10.2 percent of antimony by weight of the alloy to be used subsequently for continuous extrusion. Such an alloy may be prepared by combining a relatively pure lead, such as one of the corroding leads having at least 99.97 percent lead content, with a relatively pure antimony or a master alloy, containing, for example, about 22 percent of antimony by weight of the alloy, in desired proportions.

The combined lead and antimony mixture is then heated in accordance with the hereinabove-described method by heating above the minimum dross-melting temperature for the desired composition. The minimum dross-melting temperature for the desired composition may be obtained by reading the graph shown in FIG. 3. The heated alloy may then be cast into ingots for transportation to a place of use of the alloys in a continuous extrusion or may be used directly in the molten state for the continuous extrusion.

The melting and disappearance of the dross and the resultant specular appearance of the surface of the molten alloy, is only a guide in determining the minimum heat-treatment temperatures of lead-antimony alloys being heat treated.

Where high temperatures may be tolerated, to avoid usual observation of the surfaces of the alloy during treatment, the alloy may be heated directly to a temperature higher than that required to produce the prescribed specular surface. Such direct heating may be useful in such cases where for some reasons it is not possible to observe the surface of the alloy, or where the formation of dross is so negligible that no accurate observation might be had. For example, this may occur in cases where the alloy is molten in an enclosed kettle, or in a protective, non-oxidizing atmosphere. In such cases, the alloy may be heated either to a temperature corresponding on the graph to the composition of the alloy, or to at least 1400° F. for high purity corroding leads.

It will be understood that the above-described methods are simply illustrative of the application of the principles of the invention. Other methods may be devised by those skilled in the art which will embody the principles of the invention and fall within the spirit and scope thereof.

What is claimed is:

1. The method of preparing and using a lead-antimony alloy for continuous extrusion, which comprises:

combining and heating a pure lead having at least 99.97% lead content with antimony to obtain a lead-antimony alloy in a molten state consisting of from about .05% to about 10.2% of antimony by weight of alloy, the balance being lead,

heating the molten alloy to such a relatively high temperature in a range of from about 1000° F. to about 1400° F. that dross formed on top of the molten alloy at lower temperatures and including primarily oxides of lead and antimony disappears and the surface of the molten alloy takes on a specular appearance,

thereafter reducing the temperature of the molten alloy to a pre-extrusion temperature of from about 700° F. to about 800° F., and continuously extruding the heat-treated lead-antimony alloy over a cable core.

2. The method of preparing and using a lead-antimony alloy for continuous extrusion, which comprises:

combining and heating a pure lead having at least 99.97% lead content with antimony to obtain a lead-antimony alloy in a molten state consisting of from about .05% to about 10.2% of antimony by weight of alloy, the balance being lead,

heating the molten alloy to such a relatively high temperature in a range of from about 1000° F. to about 1400° F. that dross formed on top of the molten alloy at lower temperatures and including primarily oxides of lead and antimony disappears and the surface of the molten alloy takes on a specular appearance,

casting the heated alloy into ingots, heating the ingots to a pre-extrusion temperature of from about 700° F. to about 800° F., and continuously extruding the heat-treated alloy about a cable core.

References Cited in the file of this patent

UNITED STATES PATENTS

1,950,388      Betterton et al. ----- Mar. 13, 1934  
2,044,763      Bouton et al. ----- June 23, 1936